

Sept. 26, 1944.

H. CORTEEN

2,359,086

TREATMENT OF TEXTILE MATERIAL

Filed Dec. 27, 1940



FIG. 1



FIG. 2

Inventor  
Hansy Corteen  
By Knight, Bry  
attorneys

## UNITED STATES PATENT OFFICE

2,359,086

## TREATMENT OF TEXTILE MATERIALS

Harry Corteen, Manchester, England, assignor to  
 Tootal Broadhurst Lee Company, Limited,  
 Manchester, England, a British company

Application December 27, 1940, Serial No. 371,881  
 In Great Britain February 1, 1940

6 Claims. (Cl. 2—143)

The present invention relates to the treatment of textile materials, and more particularly to the production of a crease line therein.

It is desirable that articles such as pleated fabrics, collars, and cuffs should have a permanent line or lines along which the fabrics readily fold so that the original creases can be easily reproduced, for example by pressing or ironing during laundering.

It has previously been proposed to form a crease-line by varying the number of threads in or about the line or by differential application of acid which may or may not be followed by pressure.

The present invention consists in a method of forming a fabric having a tendency to fold along a predetermined line in which a viscous liquid containing a film-forming stiffening agent is applied to an area along and including both sides of a desired crease-line, and then applying mechanical pressure to the folded fabric first to the crease and then to the remainder of the fabric to expel more of the stiffening agent from the crease-line than from the adjacent areas on either side.

The stiffening agent is preferably applied by the use of a viscous liquid containing a polymerized material with or without a plasticising agent. Thermosetting resins are especially valuable materials. The stiffening agent may be applied to one face only of the fabric.

The linear gap of less stiffened material in the case of a collar is preferably less than 0.25 cm. and is usually between 0.10 and 0.17 cm. Although we may treat the whole surface, we prefer to stiffen a local area on either side of the crease-line the depth of which local area is less than half the height of the collar when folded and preferably less than 1½ cm. e. g. about 1 cm.

A suitable amount of film-forming solid is such as will give to the treated areas of the fabric a weft flexural rigidity at least twice and usually three to four times that of the weft of the less treated linear gap.

The film-forming solid must be such as produces a stiffening effect at normal temperatures after application to the cloth. Suitable solids include synthetic polymers which are hard rather than rubber-like and which usually have a molecular weight greater than 50,000; for example, we include the use of highly polymerised vinyl acetate and mixtures of highly polymerised vinyl acetate with polymethylmethacrylate. We prefer, however, to use far-condensed thermo-setting resinous substances such as those produced by

condensing urea and formaldehyde in presence of a catalyst for a sufficiently long time to form a non-crystallisable colloid.

The film-forming solid, e. g., in the form of a dispersion or solution is applied to the part of the cloth where the fold is to be produced together with the adjacent areas, for example by spreading it on one face of the cloth only, and subsequently to fold the textile fabric so that the film-forming material lies inside the fold. We then apply pressure with or without heat preferably in a direction at right angles to the crease; for example, by folding the fabric along the crease-line and then either passing the creased fabric laterally through a mangle, crease first, or hot ironing it crease first, in a direction at right angles to the crease-line, or squeezing it between hinged plates as hereinafter described. This application of pressure helps to expel the majority of the forming material from the actual crease-line and is assisted by the thickness of the folded cloth at this point. This effect is greatly improved by choosing a film-forming material of viscosity suitable to the nature of the cloth being treated. For example, when the viscosity is too great or the cloth too finely woven or the cloth contains a large amount of a filler or wax the film-forming material does not penetrate the fabric and this tends to give a rough surface finish and when the viscosity of the film-forming material is too low or the cloth too absorbent little migration from the crease-line takes place and this is also unsatisfactory. Liquids of suitable viscosity penetrate into the fabric but not through to the other face or into the fibres of the fabric; however, ancillary components of the film-forming material such as plasticisers or solvents may do so. The stiffening agent may also be applied as a solid with hot pressing.

We prefer to apply the film-forming material in the form of a liquid having a viscosity of not less than about 1400 c. g. s. units. In some cases the viscosity of the liquid may be increased by the addition of ammonium oleate or stearate but this tends to darken on being heated and this is undesirable. We prefer, therefore, to increase the viscosity of the liquid by other means, for example, by increasing the degree of polymerisation of the materials. In the case of urea-formaldehyde condensation products this may be done by adjusting the time allowed for condensation in presence of a catalyst and using excess formaldehyde, preferably largely in the form of paraformaldehyde to avoid excessive bulk. We have found that whilst as is well-known the preliminary con-

densation is preferably carried out in presence of alkali, a second partial condensation should be carried out in presence of an acid catalyst to reach a stage in which the liquid is highly viscous. The molecular ratio of formaldehyde to urea during these condensations should not be less than 3:1, since this ensures that the resulting viscous solution remains stable to the amount of acid catalyst which it is necessary to have present during subsequent heating to a high temperature to insolubilise the film-forming material after application to the cloth.

We have found that the final stiffness of the cloth can be varied by adding a plasticiser, in amount varying according to the degree of stiffness required; this plasticiser by acting as a diluent controls the amount of urea formaldehyde resinous material applied to the cloth. The presence of a suitable plasticiser also prevents the film-forming material from accumulating on parts of the machine which is used for applying it to the fabric.

Where the film-forming solid is applied to the textile fabric from solution, for example, in an organic solvent such as toluene in the case of polyvinyl acetate and polymethylmethacrylate mixtures, the application of the material should be followed by drying at a temperature sufficient to evaporate the solvent.

It is preferred to apply the film-forming material to one face only of the cloth and the cloth may be treated for example with a suitable amount of filler or wax to prevent undue penetration of the solid through to the other face.

The film-forming material may be applied to the whole of the textile fabric especially where the invention is applied to the manufacture of stiff or semi-stiff collars.

Titanium di-oxide or some other filler or colouring matter may be added to the liquid.

The following is an example of the preparation of a suitable urea formaldehyde condensation product and its application to the textile material.

#### Example

60 g. of urea is dissolved in 48 cc. of neutral 40% aqueous formaldehyde, 18 cc. of concentrated ammonia (sp. g. 0.88) added. After the urea has dissolved 94.8 g. of paraformaldehyde is added. The molecular ratio of urea to formaldehyde in this mixture is 1:3.8.

This mixture is then refluxed for 3 minutes, cooled slightly and 18 cc. of a 33½% aqueous solution of tartaric acid together with 0.15 g. of o-cresol (to prevent the formation of a skin) added and refluxing continued for 15 minutes by heating in an oil bath whose temperatures is 140—160° C. This mixture is then neutralised with caustic soda solution of spec. gr. 1.315 (approximately 10 cc. will be required) whilst still refluxing and the mixture subsequently cooled to room temperature. This is a highly viscous mixture.

To 40 cc. of this mixture is added 2.4 g. of solid tartaric acid and 60 cc. of Sextol (registered trade-mark) phthalate, and this mixture is stable over a reasonable period of time and is suitable for application to the textile material. Sextol is a mixture of the three isomeric methyl cyclohexanols and the phthalate of Sextol is an efficient plasticiser for the purpose of the present invention. Moreover its viscosity is such that its addition does not substantially alter the viscosity of the urea formaldehyde condensation product.

The film-forming mixture made in this way is applied to the inner face of a collar blank along the area of foldover by means of a machine embodying a take-up roller, the amount applied to the cloth being controlled by a doctor-blade.

Without allowing the mixture to dry the collar is folded along the desired line and pressed between hinged iron plates, the folded collar being placed during pressing with the crease towards the hinges thus enabling pressure to be applied to the crease line of the collar momentarily before it is applied to the remainder of the collar. In this case the plates are heated so that the squeezing and the insolubilisation takes place in a single operation, whilst the collar is still folded. This does not lead to sticking between treated areas. Alternatively, if the plates are not heated, the insolubilisation is carried out as a separate heating process. In the above example the amount of solid left on the cloth, after heating, was 17.6% calculated on the weight of cloth actually treated.

After treatment the collar has a permanent line along which it folds readily and this effect is very fast to normal laundering processes. With a typical 2-ply collar cloth a suitable amount of urea-formaldehyde film-forming material to be applied to the cloth would be between 10 and 25 mgms. per square centimetre of cloth.

The invention may be applied to textile materials other than woven fabrics.

The invention includes the manufacture in this way of pleated or creased fabrics and the treatment of collars and cuffs to obtain a crease-line so that the pleats or crease-lines can be easily found and accurately ironed. The invention is especially suitable for use in manufacturing a collar in which the curve in the plane of the collar is produced according to the method described in application No. 512,316. In this case, treatment according to the present process is carried out first so that the collar is creased before the production of the curve. Subsequently when the curve has been produced and the collar laundered the crease-line is in its correct curved form and the danger of losing the curved crease-line through subsequent washing and ironing is avoided.

An embodiment of the invention is illustrated in the accompanying drawing in which—

Figure 1 is a plan view of a collar before folding, and

Figure 2 is a diagrammatic elevation, with parts in section, showing the treated collar folded over and being pressed down more tightly at the fold edge to displace the stiffening material therefrom toward the adjacent portions of the collar.

In Figure 1 of the accompanying drawing 1 is the inner and 2 is the outer portion of a semi-stiff collar. 3 is the linear less stiffened area forming the fold line and 4 and 5 are the more stiffened areas.

Figure 2 shows the treated and folded collar 1 and 2 having the less stiffened fold line 3 and the more stiffened areas 4 and 5 being pressed between the heated iron plates A and B hinged together at C so that when pressure is applied as indicated by the arrow, the fold line is subjected to a greater pressure than the areas away from the fold line, whereby the stiffening material is partly discharged from the fold line toward the adjacent areas to provide the reduced stiffness described at the fold line. The plate A in the diagram is assumed to be of considerable length,

and extended, for example at D, for increased stability.

I declare that what I claim is:

1. A method of forming a fabric having a natural tendency to fold along a predetermined line which comprises applying a viscous liquid containing a film-forming stiffening agent to an area along and including both sides of a desired fold-line applying mechanical pressure to the folded fabric to expel more of the stiffening agent from the crease-line than from the adjacent areas on either side, and solidifying the stiffening agent on the fabric.

2. A method as claimed in claim 1 in which the stiffening agent is applied to one face of the cloth only.

3. A method of forming a fabric having a tendency to fold along a predetermined line in which a film-forming stiffening agent is applied to an area along and including both sides of a desired crease-line and then mechanical pressure is applied to the folded fabric first to the crease and then to the remainder of the fabric to expel more of the stiffening agent from the crease-line than from the adjacent areas on either side.

4. A method of forming a collar having a natural tendency to fold along a predetermined crease-line which includes the steps of applying

a water-fast film-forming stiffening agent to part only of the inner face only of a collar blank in a local area containing the proposed fold line, folding the blank along said fold line so that the film-forming agent lies inside the fold, applying mechanical pressure to the folded blank in such manner as to expel more of the stiffening agent from the fold line than from the adjacent areas on either side, and solidifying the stiffening agent on the blank.

5. A textile material having a pre-creased fold line containing a small proportion of a deposit of water-fast film of solid stiffening agent bordered on each side thereof with a similar deposit in increased proportion, whereby the textile material exercises a tendency to fold repeatedly along its pre-creased fold line.

10 6. A collar of textile fabric having a pre-creased fold line and bearing a water-fast film 15 of stiffening agent on the inner surface of the fabric along a local area near and including said fold line, said water-fast film of stiffening agent being present in a small proportion at the fold line and in larger proportions in the areas to 20 either side of the fold line, whereby the collar 25 exercises a tendency to fold repeatedly along its pre-creased fold line.

HARRY CORTEEN.